

## UNITED STATES PATENT OFFICE

2,235,508

PROCESS FOR PRODUCING ALLOYS  
CONTAINING ZIRCONIUM

Helmut von Zeppelin, Bitterfeld, and Ludwig Teichmann, Leverkusen-I. G. Werk, Germany, assignors, by mesne assignments, to Walther H. Duisberg, New York, N. Y.

No Drawing. Application January 18, 1940, Serial No. 314,451. In Germany January 24, 1939

4 Claims. (Cl. 75—177)

This invention relates to the production of alloys containing zirconium.

The production of alloys containing zirconium by standard methods, e. g. by introducing zirconium metal in pulverulent form, into a molten charge of the base metal is, because of the tendency of zirconium metal powder to ignite, only feasible when operating in an inert atmosphere or in vacuo, and even then only with considerable precaution. Moreover, commercial zirconium metal frequently contains a certain percentage of impurities such as hydrogen, oxygen, and nitrogen (the latter two generally in the form of oxides or nitrides), which impurities become incorporated in the zirconium metal in the course of its production on its being separated from reaction residues, which is generally effected by a treatment with acids. When employing zirconium metal containing the aforesaid impurities, for alloying purposes, we have observed that the alloying proceeds very slowly, so that it is desirable to use a zirconium metal for alloying purposes in which the aforesaid impurities are absent.

It is an object of our present invention to provide a process for the production of alloys containing zirconium which is not attended with the aforesaid disadvantages, i. e. which will enable the alloying operation to proceed smoothly and more rapidly and without undue oxidation of the zirconium metal.

In our copending application S. N. 314,450, entitled Production of zirconium metal, and filed on even date herewith, we have disclosed and claimed a process for the production of zirconium metal, wherein a mixture comprising a quantity of zirconium chloride, a quantity of an alkali metal chloride by weight at least about equal to half the charge of zirconium chloride, and further a quantity of magnesium metal is heated, so as to cause reduction of the zirconium chloride by the magnesium, whereupon the saline melt is separated from the zirconium metal produced.

We have now ascertained that the mixtures obtained as a result of the reaction described in our copending application, which mixtures comprise zirconium metal in pulverulent form and a saline residue comprising magnesium chloride and an alkali metal chloride, are a very efficient means for producing alloys containing zirconium.

According to our present invention reaction mixtures of the kind obtained in the process of our copending application which thus essential-

ly comprise a saline residue of magnesium chloride and an alkali metal chloride, and finely divided zirconium metal distributed therein, are directly contacted with the molten base metal of the zirconium alloy to be formed. The reaction mixture may be employed with the saline residue either fused or solidified. When employing the former alternative, then the fused saline residue containing the zirconium metal in suspension is simply poured on the molten base metal and carefully stirred thereinto. It is, however, always preferable first to allow the zirconium metal produced by the reaction to settle from the fused saline residue and then to discard the bulk of the latter so that only that portion of the mixture which contains the zirconium metal in somewhat concentrated form is used for alloying purposes. The separation of the bulk of the saline residue from the portion containing the settled zirconium metal may be effected either by decanting the fused saline residue off the said part, or by allowing the entire reaction mixture to solidify after settling, whereupon the cake is divided into the aforesaid two portions, e. g. by cutting. The cake can then be broken up and strewn on and carefully stirred into the molten base metal. The saline residue introduced along with the zirconium metal forms a covering on the alloy which protects the latter from undesirable reaction with the constituents of the atmosphere, and incidentally also serves as a flux; the dissolution of the zirconium metal in the base metal is thus enabled to take place with the greatest rapidity.

The efficiency of the reaction mixtures containing zirconium metal and produced in accordance with our copending application, for alloying purposes, is probably due to the fact that any reaction of the zirconium metal such as oxydation is prevented by the particles of zirconium metal being and remaining completely surrounded by the saline residue until the zirconium is taken up by the base metal.

## Example

1.5 kgs. of a reaction mixture produced in accordance with our copending application S. N. 314,450 and consisting of 33.4% by weight of potassium chloride, 33.4% by weight of magnesium chloride and 29.4% by weight of zirconium metal particles, balance impurities, are introduced into 20 kgs. of a zinciferous magnesium base alloy heated to 770° C., while stirring. The stirring is continued for about 1 minute thereafter, whereupon the whole is allowed to settle.

The molten metal is then poured while keeping back the slag, and the alloy obtained then contains 0.5% of zirconium.

We claim:

- 5 1. A process for producing alloys containing zirconium, which comprises causing to contact with the molten metal to be alloyed with zirconium, a product consisting of finely divided particles of zirconium metal dispersed in a mixture of magnesium chloride and an alkali metal chloride.
- 10 2. A process for producing alloys containing zirconium, which comprises causing to contact with the molten metal to be alloyed with zirconium, a product consisting of finely divided particles of zirconium metal dispersed in a mixture of magnesium chloride and an alkali metal chloride, said product having been produced by reaction of zirconium chloride with magnesium in the presence of said alkali metal chloride.
- 15 3. A process for producing alloys containing

zirconium, which comprises introducing, while carefully stirring, into the molten metal to be alloyed with zirconium a product consisting of finely divided particles of zirconium metal dispersed in a mixture of magnesium chloride and an alkali metal chloride, said product having been produced by reaction of zirconium chloride with magnesium in the presence of said alkali metal chloride.

4. A process for producing a magnesium base 10 alloy containing zinc and zirconium, which comprises introducing, while carefully stirring, into the liquid alloy of magnesium and zinc, a product consisting of finely divided particles of zirconium metal dispersed in a saline melt of magnesium chloride and an alkali metal chloride, said product having been produced by reaction of zirconium chloride with magnesium in the presence of said alkali metal chloride.

HELMUT VON ZEPPELIN. 20  
LUDWIG TEICHMANN.